

# United States Patent

Byrne

[15] 3,649,795

[45] Mar. 14, 1972

[54] ELECTRICAL CONTACTS

[72] Inventor: William Ralph Byrne, 722 Harris Avenue, Providence, R.I. 02409

[22] Filed: May 1, 1969

[21] Appl. No.: 820,849

[52] U.S. Cl. .... 200/166 C, 29/199

[51] Int. Cl. .... H01h 1/02

[58] Field of Search ..... 29/199; 200/166 C; 174/133 R

[56] References Cited

UNITED STATES PATENTS

2,064,998 12/1936 Waite ..... 200/166 C  
2,379,641 7/1945 Keitel ..... 200/166 C

2,812,406 11/1957 Egan ..... 200/166 C

OTHER PUBLICATIONS

Product Design Catalog File, Sweet's Catalog Service, F. W. Dodge Corp., N.Y., N.Y., 1960, pgs. 6 and 7, Section 2c/Sy.

Primary Examiner—L. Dewayne Rutledge

Assistant Examiner—J. Davis

Attorney—Burns, Doane, Swecker & Mathis

[57] ABSTRACT

An electrical contact comprising a high-purity nickel alloy for use in a corrosive atmosphere as, for example, in the presence of sulphur bearing materials.

5 Claims, 4 Drawing Figures



PATENTED MAR 14 1972

3,649,795

Fig. 1.



Fig. 2.



Fig. 3.



INVENTOR

*W. RALPH BYRNE,*

*Attorneys, BY Moore, Bennett, Sander & Mathis*

ATTORNEYS

## ELECTRICAL CONTACTS

## SUMMARY OF THE DISCLOSURE

In the electrical contact industry, it is important to use contact materials which have a stable contact resistance.

The reaction of the contact material with its environment can cause a reaction product on the surface of the contact. Many of these reaction products are insulators or poor conductors of electricity. The formation of these high resistance

other apparatus which require a stable contact resistance in a corrosive environment.

An electrical contact according to the invention is exceptionally free from non-metallic inclusions, has a low base hardness and good ductility which will permit heavy cold deformation without reannealing.

An example of the chemical composition of the alloy for use as an electrical contact according to the invention is given below in percentages by weight:

|                | Ni    | C   | Mn    | Fe   | Cu    | Cr    | S     | Si    | Mg    | Ti    | Co    |
|----------------|-------|-----|-------|------|-------|-------|-------|-------|-------|-------|-------|
| Nominal.....   | 99.98 | .01 | <.001 | .001 | <.001 | <.001 | <.001 | <.001 | <.001 | <.001 | <.001 |
| Limiting ..... | 99.97 | .02 | .001  | .005 | .001  | .001  | .001  | .001  | .001  | .001  | .001  |

\* Maximum except nickel, which is minimum.

or insulation materials on the surface of the electrical contact material will cause a high contact resistance and if this surface layer is especially insulating, it can even prevent the flow of current through the contact.

As an example, if copper is used as a contact metal, sulphur or oxygen in the atmosphere will react to form copper sulphide or oxide on the oxide on the surface of the copper. This layer of sulphide or oxide on the surface of the copper will then either cause a high contact resistance or, if the layer is thick enough, it can prevent the flow of current across the contacts and thus cause an open circuit.

Attempts have been made heretofore to use commercially available alloys of nickel as contact materials, but these did not show an especially stable contact resistance.

I have discovered that a high purity grade of nickel alloy containing at least 99.9 percent of pure nickel and not more than 0.1 percent of impurities has unique properties as a contact material which make it ideally suitable for low voltage and low current applications. The unique property of this alloy is its stable contact resistance which has not been found in other nickel alloys with a lower nickel content. This alloy will maintain a low stable contact resistance in the presence of sulphur bearing materials as, for example, hydrogen sulphide, aluminum sulphide, sulphur dioxide, or pure sulphur, which would cause the formation of metal sulphides with commercial nickel alloys. This fact makes the new contact very suitable for low voltage and low current work.

## BRIEF DESCRIPTION OF DRAWINGS

I have illustrated an application of this invention in the accompanying drawings, in which:

FIG. 1 is a top plan view of a contact board having a plurality of contacts imbedded therein;

FIG. 2 is a cross section therethrough; and

FIGS. 3 and 4 are diagrammatic sectional views showing stator contacts.

## DETAILED DESCRIPTION OF DRAWINGS

In the preparation of an electrical contact embodying this invention, I use a high purity nickel alloy which has a purity of not less than 99.9 percent, and preferably 99.98 percent, of nickel. This alloy is initially formed as wire which can be drawn down to a thin strip and flattened to approximately 0.015 inch thick by 0.061 inch wide in a continuous strip. The flattened alloy wire can be fabricated or used as needed as an electrical contact.

As illustrated, for example, in FIG. 1, a contact board is indicated generally by the numeral 1. This is of any suitable or desired construction and size according to the use to be made thereof. In this embodiment, the contact board is molded of plastic and has imbedded therein a suitable number of electrical contacts in accordance with the invention, generally indicated at 2, projecting transversely through the board. In this embodiment, the contact board is used as a part of a rotor contact in a television tuner. Electrical contacts according to the invention may also be used in computers, switches, rotor switches, telephone relays, telephone connectors and in any

This alloy is extremely malleable by metal working techniques, i.e., mechanical deformation. Softness is also an important characteristic of contact materials. The softness characteristic is important for electrical contact purposes in that the contact mechanically deforms easily to increase the actual area of contact, thereby lessening the electrical resistance.

The use of an electrical contact made wholly of the alloy has economical advantages over plated or clad materials.

Sulphides, ozone, and oxygen in the atmosphere around the contacts are particularly damaging to electrical contacts in that they are highly reactive and form insulating films on the contact metal. Ozone is created as a result of the arcing which normally accompanies the making and breaking of electrical contacts and is continuously being created in an operation where there is a voltage across the contacts when they open or close.

The high volume conductivity is important for contacts for use in apparatus such as computers and telephone switches or in applications where the current is high and  $I^2R$  heating becomes noticeable. The high volume conductivity is as important for television tuner contacts, because actual total resistance can be adjusted or compensated for in a television tuner circuit.

It is also possible to use the high purity nickel alloy as the upper surface of a flexible contact of multiple layers as, for example, over a layer of base metal to prevent atom migration. Examples thereof are shown in FIGS. 3 and 4.

The strip shown in diagrammatic cross section in FIG. 3 may be used as a stationary contact for television tuners. The major portion of the thickness of the strip is of base metal, indicated at 3, having a relatively thin layer of silver alloy coated on the surface thereof, as indicated at 4. The silver alloy is used primarily because of its electrical conductivity. Only a thin surface layer of silver alloy is used because the high frequency current which is used only travels on the surface. A gold alloy contact element is indicated at 5 embedded in the surface of the silver layer 4.

In FIG. 4, a high purity nickel alloy is used as the base metal, indicated at 6, with the gold alloy contact 7 embedded in the surface thereof.

In actual use a problem is encountered in that the silver atoms migrate across the surface of the gold alloy (by surface diffusion). These silver atoms on the surface of the gold are then chemically attacked by sulphur bearing compounds in the atmosphere and form a black silver sulphide on the surface of the gold. The silver sulphide then acts as a resistance barrier to the flow of current across the contacts, and gives non-uniform tuning of the television picture.

I have discovered that by replacing the silver alloy 4 with high purity nickel alloy will eliminate the surface diffusion problem.

I have also discovered that the strip having the configuration shown in FIG. 4 makes a good stator material, and it is easier and less costly to manufacture. The base material for this strip may be 99.5 percent nickel to 99.8 percent nickel. It is important, however, that the strip be manufactured so as to give good fatigue properties.

An electrical contact embodying the invention of a high purity nickel alloy (between 99.9 and 99.98 percent nickel) may be used with advantage for medium energy contacts (from 1 to 15 amps) and is a good replacement for commercially pure silver and silver alloys. This has been found to be especially useful up to 15 amps.

I claim:

1. An electrical contact for use for low energy application with low contact resistance in a corrosive atmosphere comprising a stable alloy of highly pure nickel in excess of 99.9 percent.

2. An electrical contact according to claim 1, wherein the stable alloy has a nominal purity of 99.98 percent nickel.

3. An electrical contact according to claim 1, wherein the alloy forms a solid contact body.

5 4. An electrical contact according to claim 1, comprising a substantially flat wire of highly pure nickel having a purity of substantially 99.98 percent.

10 5. An electrical contact according to claim 1, wherein the stable alloy has a nominal purity of 99.98 percent pure nickel and not to exceed 0.02 percent of impurities.

\* \* \* \* \*

15

20

25

30

35

40

45

50

55

60

65

70

75